

## UNITED STATES PATENT OFFICE

2,428,829

## SMOKELESS POWDER

Ernst Berl and Walter George Berl, Pittsburgh,  
Pa.; Walter G. Berl as executor of Ernst Berl,  
deceased

No Drawing. Application February 26, 1942,  
Serial No. 432,482

4 Claims. (Cl. 52—5)

1

Until now two types of smokeless powders have been used for military and civilian purposes. One category is composed of mixtures of cellulose nitrates (nitrocelluloses) with nitrogen contents from 12.3 up to 13.6%. Those mixtures contain completely or partly ether-alcohol-soluble collodion wools (12.0—12.6% nitrogen) plus a certain amount of ether-alcohol insoluble guncotton (13.0—13.6% nitrogen). They can be obtained with mixed acids composed of nitric acid, sulphuric acid, water. They have to undergo a stabilizing process. These mixtures of collodion wool and guncotton are treated with ether-alcohol. The ether-alcohol-insoluble guncotton fibers are imbedded in the gel resulting from ether-alcohol-soluble collodion wool. In this way one can get brisant smokeless powders because the non-dissolved guncotton fibers burn with greater speed than the homogeneous colloid formed from ether-alcohol-soluble collodion wool. Other smokeless powders of this type are made from guncotton (13.0—13.3% N) by complete gelatinization with acetone. They represent the so-called "mild" smokeless powder type.

A second class of smokeless powders is produced by a mixture of cellulose nitrate (nitrocellulose) with glycerine trinitrate (nitro-glycerine) with or without glycol dinitrate (nitro-glycol). In adding the liquid nitric acid esters of organic alcohols to solid cellulose nitrates, one raises the nitrogen content, and, therefore, the oxygen content present as  $\text{NO}_2$ -oxygen (active oxygen). In this way it is possible to obtain smokeless powder with more energy and better ballistic properties than has been obtained until now with pure cellulose nitrate smokeless powders with a collodion wool basis.

Those glycerine trinitrate (glycol dinitrate)-cellulose nitrate smokeless powders can be produced without using a common volatile solvent for the used lower nitrated cellulose nitrates and glycerine trinitrate (glycol dinitrate). Then the "ballistites" result which are ballistically stable. For those smokeless powders cellulose nitrates of the collodion type (with maximum nitrogen content of 12.6%) have to be used. At elevated temperatures and pressure, they form with the nitrated aliphatic alcohols (glycerine trinitrate and glycol dinitrate) a gelatine. The fiber structure of the cellulose nitrate in this gel is completely destroyed. In view of the very hot flames produced by smokeless powders of this type containing larger amounts—up to 50%—of glycerine trinitrate (glycol dinitrate), usually the quantity of those liquid nitric acid esters of aliphatic

2

alcohols has to be reduced to 20 or 25%. Then the complete gelatinization of cellulose nitrate (nitrocellulose) fibers at elevated temperature and elevated pressure without using volatile solvents for both esters is rather difficult to carry out. Many accidents happen then unless larger quantities of stabilizers which, like derivatives of urea, such as diethyl diphenyl urea, urethane, etc., in molten state are solvents for collodion wools are added. By this additional material the ballistic properties of such a smokeless powder are reduced.

In using a common solvent, for instance acetone, or guncotton (alcohol-ether-insoluble higher nitrated cellulose) and for glycerine trinitrate (glycol dinitrate), the use of higher nitrated material (12.7—13.3% N) is possible. Those smokeless powders—cordites—can be produced without greater danger. They have the disadvantage that the necessary elimination of the used volatile solvent (mostly acetone) presents sometimes dangerous complications. The resulting cordites are often ballistically unstable. They retain larger quantities of solvents, lose those during storage, and after a longer period of storage become more brisant.

We have found that stable cellulose nitrates which can be produced from cellulose with mixtures of water-free nitric acid and phosphoric acid (ortho- and metaphosphoric acid) containing several percent of free phosphoric acid anhydride, called superphosphoric acids, or those cellulose nitrates which produced from cellulose with mixtures of glacial acetic acid and 100% nitric acid without or with a certain amount of either acetic anhydride or phosphoric acid anhydride, according to the U. S. patent application 385,580, filed March 27, 1941, of Ernst Berl (now U. S. Patent No. 2,384,415 of September 4, 1945), can be used with great advantage for the production of smokeless powders.

We have furthermore found that those highest nitrated cellulose nitrates can be produced from already nitrated lower cellulose nitrates obtained by nitration with mixed acids composed of sulphuric acid, nitric acid and water by additional nitration with mixed acids composed of water-free nitric acid and superphosphoric acids, or glacial acetic acid, with or without addition of acetic anhydride or phosphoric acid anhydride.

These new types of pure cellulose nitrate smokeless powders contain practically the same amount of nitrogen as those smokeless powders composed of 80—76% of collodion wool with

12.0-12.6% N and 20-25% of glycerine trinitrate (glycol dinitrate).

Those highly nitrated, stable cellulose nitrates can be produced with nitrogen contents of more than 13.3% and up to 14%. The following table shows the nitrogen content of mixed cellulose nitrate-glycerine trinitrate smokeless powders whereby cellulose nitrates with different nitrogen contents and different ratios between cellulose nitrate and glycerine trinitrate are used.

Smokeless powders made from:

- 70 parts cellulose nitrate with 12% nitrogen content and 30 parts glycerine trinitrate with 18.5% nitrogen content contain 13.9% nitrogen and 31.8% oxygen.  
 70 parts cellulose nitrate with 12.6% nitrogen content and 30 parts glycerine trinitrate with 18.5% nitrogen content contain 14.35% nitrogen and 32.8% oxygen.  
 75 parts cellulose nitrate with 12% nitrogen content and 25 parts glycerine trinitrate with 18.5% nitrogen content contain 13.62% nitrogen and 31.2% oxygen.  
 75 parts cellulose nitrate with 12.6% nitrogen content and 25 parts glycerine trinitrate with 18.5% nitrogen content contain 14.1% nitrogen and 32.2% oxygen.  
 80 parts cellulose nitrate with 12% nitrogen content and 20 parts cellulose glycerine trinitrate with 18.5% nitrogen content contain 13.3% nitrogen and 30.4% oxygen.  
 80 parts cellulose nitrate with 12.6% nitrogen content and 20 parts glycerine trinitrate with 18.5% nitrogen content contain 13.8% nitrogen and 31.5% oxygen.

One sees from these figures that pure cellulose nitrate smokeless powders produced from cellulose nitrates with nitrogen contents up to 13.9% and 14.0% and oxygen contents between 31.8% and 32.2% equal or surpass the nitrogen and the active oxygen content of most of those smokeless powders made as ballistite powders from collodion wools and glycerine nitrate.

These new, pure cellulose nitrate (nitrocellulose) smokeless powders with ballistic performances which have not been obtained up to this time with other pure cellulose nitrate smokeless powders by using highest nitrated cellulose nitrates produced with phosphoric or glacial acetic acid nitration processes present many advantages over the "mixed" cellulose nitrate-glycerine trinitrate (glycol dinitrate) smokeless powders.

The advantages of the production of smokeless powders made from highest nitrated cellulose nitrates alone are manifold. For their production only one operation is necessary—the nitration of cellulose. This nitration can be carried out in very short time intervals of a few seconds or minutes at room temperature. The removal of the spent acid and the stabilization of the resulting highest nitrated cellulose nitrates by repeated hot extraction with swelling but not these cellulose nitrate dissolving agents like strong methyl- or ethyl-alcohol, best close to their boiling points, can also be carried out in very short time intervals. Furthermore, it is not necessary to pulp the cellulose nitrate fiber in order to carry out this stabilization process. Phosphoric acid and acetic acid do not form mixed esters with nitrated celluloses as is the case with the use of mixed acids containing sulphuric acid. Then, as is known, dangerous cellulose nitro-sulfates are formed. They are difficult to remove so that

stable cellulose nitrates may be obtained. The pulping which has to be carried out in the normal stabilization process when sulphuric acid containing mixed acids are used requires time. The costs for power for this cutting of the hardened cellulose nitrate fiber are rather high and the mechanical losses, due to the shortening of the fibers, are relatively great. All these inconveniences are eliminated by the special nitration processes producing longer fibers of highest nitrated cellulose without their pulping in order to eliminate bound or strongly adsorbed sulphuric acid.

This highest nitrated material is practically insoluble in methanol and ethanol; therefore, the yield after stabilization by hot extraction with these alcohols is high. Furthermore, it is not necessary to use afterwards a special dehydration operation for the removal of water from wet cellulose nitrates stabilized with the older stabilization processes by treatment with acidified and alkaline water. This dehydration process needs time and lowers the yield.

The production of any geometric form for smokeless powders made from this highly nitrated cellulose plus stabilizers, and other additional material for cooling the explosion flames, such as urea, nitroguanidine, etc., and optical compensation of the yellow-red combustion gases, such as potassium salts, can be made with the help of acetone and its homologues. Stabilizers, like diphenylamine or substituted urea compounds, such as diethyl diphenylurea, due to the strongly hydrophobic nature of this highest nitrated material, are retained with strong forces. The same is true for added aromatic nitro compounds like TNT and dinitrotoluene or dinitrobenzene. This fact together with the perfect stabilization by using swelling but not dissolving agents, like methanol and ethanol, allows the production of smokeless powders of until now unattained stability.

One can destroy the fiber structure of these fibrous highly nitrated cellulose nitrates by subjecting suspensions of dehydrated, highly nitrated cellulose fibers together with non-solvents, like ether-alcohol, methanol, mixtures thereof, or mixtures with acetone and higher ketones to low temperature, down to  $-70^{\circ}$  C. The lowering of the temperature causes the complete destruction of the fiber structure under formation of a perfectly gelatinized material. In bringing the temperature up to room temperature, or temperatures up to the boiling point of the used solvents, the formation of very viscous gels takes place which can be transformed by higher temperature and pressure into any geometric form.

Highly nitrated cellulose fibers insoluble at room temperature in the used solvents or solvent mixtures introduced at room temperature in this gel obtained by the aforementioned treatment at low temperature remain insoluble. One gets a gel in which the non-attacked, highly nitrated cellulose fibers are imbedded. After elimination of the solvent by evaporation or by extraction, those non-dissolved fibers remain undissolved. In this way one gets a brisant smokeless powder with until now unknown properties.

Therefore, one can produce in this way mild smokeless powders whereby the whole amount of highly nitrated cellulose fibers is converted into a gel under complete destruction of the fiber structure. One can produce also smokeless powders with different ratios between this gel and highest nitrated cellulose fibers with conserved

fiber structure. The speed of combustion in the arms can therefore be regulated at will.

The removal of the volatile solvent from the formed smokeless powder can be carried out by drying it in warm, non-inflammable gas free of or poor in oxygen. The drying can be carried out in counter current so that the already nearly dry smokeless powder comes in contact with warm oxygen-free (poor) gas containing no solvent vapors. The non-combustible gas, for instance flue gas, or nitrogen, or carbon dioxide, already charged with solvent vapors, comes in contact with the fresh smokeless powder containing larger amounts of not yet removed solvents. The drying can be carried out also in parallel stream. The fresh smokeless powder travels in the same direction as the warm drying gases. The last amounts of the solvent are retained by the smokeless powder with rather great force. They can be removed by systematic treatment with watery solutions of swelling but not dissolving substances, for example, alcohol-water solutions or dioxane-water solutions, using first solutions with a higher percentage of the organic non-solvent, for example alcohol, and at the end solutions containing no organic solvent, for example alcohol or dioxane, at all. One can add to these alcohol solutions stabilizers and substances which influence the speed of combustion, such as guanidine, so that in this way a kind of progressively burning powder could be obtained.

The production and use of smokeless powders with highest nitrogen-containing cellulose nitrate content present further great advantages over the mixed cellulose nitrate-glycerine trinitrate (glycol dinitrate) smokeless powders. It is known that the latter cannot be dried at somewhat higher temperatures; this in view of the volatility of the glycerine nitrate (glycol nitrate) which easily condenses in pure form on cooler places. It may become unstable and may be the source of explosions. Furthermore, one cannot treat those mixed cellulose nitrate-glycerine trinitrate powders during a long time with water in order to remove the last amounts of volatile solvents, especially if lower nitrated cellulose nitrates (12.0-12.6% N) with free hydroxyl groups are used. Then water displaces the otherwise strongly adsorbed glycerine trinitrate (glycol dinitrate) and causes therefore a change in the composition of the smokeless powder.

The new, pure cellulose nitrate smokeless powders, due to their strong hydrophobic nature, are practically insensitive toward humidity. Smokeless powders made from cellulose nitrates with lower nitrogen content show very strong sensitiveness toward the atmosphere with different amounts of humidity. Therefore, the ballistic properties of those older smokeless powders made from lower nitrated cellulose nitrates are inferior compared with the excellent ballistic properties of these pure cellulose nitrate smokeless powders produced from cellulose nitrates containing the highest possible degree of nitrogen and, therefore, bound active oxygen content. They show the highest degree of hydrophobia; in other words, water-repelling qualities, and do not change their ballistic properties when kept in contact with air with different amounts of humidity.

#### Example 1

Cellulose nitrate with 13% nitrogen content produced with mixed acids composed of sulfuric acid, nitric acid and water is treated with

mixed acids composed of water-free nitric acid and superphosphoric acid (pyrophosphoric or metaphosphoric acid) at room temperature or somewhat increased or lower temperature. The 5 nitrogen content after this additional nitration and after stabilization with strong alcohol is raised to 13.9-14.0% nitrogen. To the resulting wet mass acetone and 1-8% of centralite—symmetric diethyl diphenyl urea (melting point 10 71.5°C.) are added. Small amounts of potassium salts for the optical compensation may be added. The preparation of smokeless powders of any geometric form has to be carried out according to 15 known processes. The resulting smokeless powder has the same ballistic properties as ballistite to which the same amounts of centralites and potassium salts have been added. The new smokeless powder is not influenced in its ballistic 20 activity by the humidity of the air and by a treatment with water. Ballistite submitted to the same conditions would adsorb, according to the humidity of the air, larger or smaller quantities of water and by a treatment with liquid water would lose glycerine trinitrate and would change 25 its ballistic properties.

#### Example 2

Cellulose nitrate with 13.95% nitrogen content 30 produced by the direct nitration of cellulose with water-free nitric acid and superphosphoric acid (pyro- or metaphosphoric acid) or according to Example 1 is extracted and stabilized with hot methanol. Methanol does not dissolve the fiber 35 at room or higher temperature. To this now excellently stabilized material which has retained its fibrous form more methanol is added if necessary. This suspension is submitted to low temperature (-50°C.). Then the fiber structure of the nitrated cellulose disappears completely and a homogeneous gel is formed. To this gel stabilizers, furthermore substances which lower the 40 temperature of explosion, like nitroguanidine, may be added. The mixture, best under continuous mixing, has to be brought to room temperature. Its viscosity increases. Under pressure and heat the formation of smokeless powder of any 45 geometric form can be carried out.

#### Example 3

The first steps of the production of smokeless 50 powder as described in Example 2 are carried out. To this gel without fiber structure at room temperature unpulped or pulped fibrous cellulose 55 nitrated dehydrated and stabilized by methanol with nitrogen contents from 12.8-14% N is added. In appropriate kneaders a uniform suspension of these fibers in this gelatine is made. Between 60 10 and 400% of the fibrous material may be added to the gel; this based on the amount of cellulose nitrate of which the fiber structure has been destroyed.

#### Example 4

Instead of using methanol, as described in Examples 2 and 3, ether-alcohol may be used as a 65 solvent for this highly nitrated guncotton which is ether-alcohol insoluble at room temperature. At the low temperature (-20 to -70°C.) a complete gelatinization under loss of fiber structure 70 of this highest nitrated guncotton material takes place. One can add, as is described in Example 3, to this homogeneous gel at room temperature fibrous cellulose nitrate (with 12.8-14% N) in 75 order to get a more brisant smokeless powder.

*Example 5*

To methanol, as is described in Examples 2 and 3, or ether-alcohol, as is described in Example 4, small amounts of acetone are added. Then a change in the properties of the swollen mass takes place. In this way it is possible to get an emulsion whereby the cellulose nitrate is the uninterrupted phase and the solvent the discontinuous phase. In some cases this may represent a certain advantage.

*Example 6*

Acetone as used in Examples 1 and 5 may be partly or wholly substituted by higher aliphatic ketones like methyl-ethyl ketone, or methyl-propyl ketone or di-isobutyl ketone.

We claim:

1. Hydrophobic single base smokeless powder produced from a stable cellulose nitrate with nitrogen contents from 13.8 to 14.0%, comprising a gel without fiber structure in which nitrated cellulose fibers with nitrogen contents up to 14.0% and the same solvent properties as the cellulose nitrate of said gel are imbedded.
2. Hydrophobic single base smokeless powder produced from a stable cellulose nitrate with nitrogen contents from 13.8 to 14.0% according to claim 1 with the addition of an appropriate stabilizer.
3. Hydrophobic single base smokeless powder produced from a stable cellulose nitrate with nitrogen contents from 13.8 to 14.0% according to claim 1 with the addition of a cooling agent.
4. Hydrophobic single base smokeless powder

produced from a stable cellulose nitrate with nitrogen contents from 13.8 to 14.0% according to claim 1 with the addition of a substance capable of optically compensating the yellow-red combustion flames.

ERNST BERL.  
WALTER GEORGE BERL.

## REFERENCES CITED

- 10 The following references are of record in the file of this patent:

## UNITED STATES PATENTS

|    | Number    | Name      | Date          |
|----|-----------|-----------|---------------|
| 15 | 2,125,880 | Berl      | Aug. 9, 1938  |
|    | 1,938,176 | Dreyfus   | Dec. 5, 1933  |
|    | 1,884,802 | Miles     | Oct. 25, 1932 |
|    | 781,926   | Wiley     | Feb. 7, 1905  |
|    | 2,230,848 | Regestein | Feb. 4, 1941  |
| 20 | 2,153,331 | Kunz      | Apr. 4, 1939  |
|    | 2,028,990 | Olsen     | Jan. 28, 1936 |
|    | 1,978,071 | York      | Oct. 23, 1934 |
|    | 1,978,070 | York      | Oct. 23, 1934 |

## FOREIGN PATENTS

|    | Number  | Country       | Date          |
|----|---------|---------------|---------------|
| 25 | 632,614 | France        | Oct. 10, 1927 |
|    | 483,474 | Great Britain | Apr. 19, 1938 |
|    | 269,529 | Great Britain | Apr. 8, 1927  |

## OTHER REFERENCES

- Allen's Comm. Organic Analysis, 5th ed., vol. 3, p. 598,  
Explosives, (1925) Marshall, vol. 1, Phila., 1917,  
35 pp. 135-137.